

# UNITED STATES PATENT OFFICE.

PAUL C. SEEL, OF ROCHESTER, NEW YORK, ASSIGNOR TO EASTMAN KODAK COMPANY, OF ROCHESTER, NEW YORK, A CORPORATION OF NEW YORK.

## PROCESS OF DEHYDRATING NITROCELLULOSE AND REDUCING THE FIRE RISK THEREOF.

1,398,911.

Specification of Letters Patent. Patented Nov. 29, 1921.

No Drawing.

Application filed August 9, 1920. Serial No. 402,478.

To all whom it may concern:

Be it known that I, PAUL C. SEEL, a citizen of the United States of America, residing at Rochester, in the county of Monroe 5 and State of New York, have invented certain new and useful Improvements in Processes of Dehydrating Nitrocellulose and Reducing the Fire Risk Thereof, of which the following is a full, clear, and exact specification.

This invention relates to a process of handling nitrocellulose between the washing operations and the plasticizing operations. The chief object of the invention is to provide a novel step or steps by which all harmful amounts of water may be removed from the washed nitrocellulose fibers without increasing the fire risk, such fibers being kept in a condition of comparative safety up to 20 the time when they are incorporated into suitable compositions or forms. Other objects will hereinafter appear.

After cellulose fibers are nitrated, the acid is removed therefrom by washing in water 25 or aqueous solutions. But the amount of water clinging to the washed fibers cannot be reduced by wringing or like mechanical means to a point where the nitrocellulose is ready for incorporation into the usual plastic 30 compositions. While the retained moisture may be finally removed by evaporation, such a step has proven in practice to be a very dangerous one, because the hazard of fire, or even of explosion, is very greatly increased when the nitrocellulose is dry. For 35 safety during the entire period of storage and transport, the nitrocellulose should be kept in a wetted condition, the term wetted applying herein to fibers intermingled with 40 non-aqueous liquids as well as when intermingled with water.

In order to remove the water and at the same time keep the nitrocellulose fibers safely wetted a suitable liquid should be 45 allowed to percolate through the mass of fibers and absorb the remnant of moisture which remains intermingled therewith after the washing and wringing operations. The liquid thus used should be a non-solvent of 50 the nitrated cotton, under the conditions prevailing during the percolation and should also be capable of taking up or absorbing the water within itself without harm. After the percolation has taken 55 place and the water has been absorbed, the

excess of liquid is removed, leaving enough liquid intermingled with the fibers of nitrocellulose to keep the latter suitably wetted for fire prevention.

I have found that effectively anhydrous 60 normal butyl alcohol and effectively anhydrous isobutyl alcohol and a mixture of them have each the necessary properties for successful use in the above described operations. Moreover, because of the low volatility of these liquids, the amount of them which is left on the fibers will keep the latter sufficiently wetted to minimize the fire hazard over a considerable period of time during storage and transportation prior to the 70 final use of the fibers. These alcohols even in the ordinary commercial grades have the property, when suitably dehydrated, of taking up a considerable amount of water without harm to themselves or subsequent products. By effectively anhydrous I, therefore, mean that sufficient water has been removed from these alcohols by usual dehydrating methods prior to percolation to enable them to absorb a useful amount of water when 80 intermingled with moist nitrocellulose fibers. Of course, the commercial grades of these alcohols may contain small amounts of other substances without impairing their effectiveness. Both of these alcohols boil above 100 85 degrees C. and I generically designate them as butylic alcohols of low volatility.

I will now describe, by way of illustration, the preferred embodiment of my invention. The fibers of nitrocellulose, moist with the 90 final wash water, are mechanically treated, as in a centrifuge, to press or wring out as much water as possible, the water remaining being, for example, from forty to sixty per cent. by weight of the nitrocellulose. 95 Normal butyl alcohol of the commercial grade (comprising in typical samples over eighty per cent. of this alcohol and boiling approximately at 115 to 117 degrees C.) is then thoroughly percolated through the 100 mass. The amount of such alcohol that can be employed depends on the degree to which it has been dehydrated. In ordinary practice the amount of butylic alcohol employed, when well dehydrated, is for example from 105 five to ten times the weight of nitrocellulose to be treated. After the water has been absorbed, by the percolated liquid, the excess of alcohol is removed mechanically, say in a 110 centrifuge. This removal may be carried to

the point where the amount of normal butyl alcohol remaining on the nitrocellulose fibers becomes, for instance, forty to sixty per cent. by weight of the latter. Of course any 5 other safe per cent. could be retained. The nitrocellulose, thus wetted by this retained alcohol, can be kept in storage or transported with low fire risk for a considerable 10 length of time, the normal butyl alcohol being of a usefully low volatility, and consequently remaining in place on the fibers. Isobutyl alcohol either alone or in admixture 15 with normal butyl alcohol can also be used in the same way.

15 Having thus described my invention, what I claim as new and desire to secure by Letters Patent is:

1. In the process of preparing nitrocellulose, the step which comprises treating nitro- 20 cellulose carrying water, with a liquid comprised chiefly of effectively anhydrous butyl alcohol of low volatility.

2. In the process of preparing nitrocellulose, the step which comprises treating nitro- 25 cellulose carrying water with effectively anhydrous normal butyl alcohol.

3. The process of treating nitrocellulose fibers which comprises the steps of washing the same, mechanically removing the excess of water, percolating through the mass of 30 said fibers a liquid comprising chiefly an effectively anhydrous butyl alcohol of low volatility, and removing part of said alcohol.

4. The process of treating nitrocellulose fibers which comprises the steps of washing the same, mechanically removing the excess of water, percolating through the mass of 35 said fibers sufficient effectively anhydrous normal butyl alcohol to absorb the water remaining with the fibers, and removing the 40 excess of said alcohol from the fibers, the remaining alcohol intermingled with the fibers, reducing the fire risk.

5. In the process of preparing nitrocellulose, the step which comprises treating one 45 part of nitrocellulose fibers carrying forty to sixty per cent. of water with from five to ten parts of commercial anhydrous normal butyl alcohol.

Signed at Rochester, New York, this 2nd 50 day of August, 1920.

PAUL C. SEEL.